

## UNITED STATES PATENT OFFICE

1,930,646

## METHOD OF IMPREGNATING POROUS MATERIALS

Philip P. Gray, Hollis, N. Y., and Ernest E. Werle, Grantwood, N. J., assignors to The Fibre Conduit Company, Orangeburg, N. Y., a corporation of New York

No Drawing. Application November 12, 1930  
Serial No. 495,287

2 Claims. (Cl. 91—70)

This invention relates to impregnating porous material, such as fiber or pulp, with bituminous compounds such as asphalt, pitch, and the like for waterproofing, insulating, and similar purposes.

More particularly, the invention includes a method of treating formed bodies, such as duct or conduit, made of cellulosic fiber or pulp for the purpose of rendering the bodies waterproof, and maintaining their good insulating properties for electrical wiring underground, or in the floors or walls of buildings, or in the open air. The principles of the invention are, however, applicable quite broadly to the impregnation of such materials or objects regardless of the use to which they are to be put.

The impregnating substances which we have employed, and as to which the invention is particularly pertinent, are substances such as pitch, which may be of quite varied and even complex composition or mixture, but which in any case are susceptible of being melted at an elevated temperature, and on cooling to normal temperatures will assume a substantially solid or approximately non-fluid state.

For the purpose of clear illustration, but without limiting the invention thereto, we shall refer to the treatment of fiber conduit or duct made of wood pulp or newsprint pulp with pitch, such as for example, that known in the trade as "water gas tar pitch". Such duct is usually molded of the pulp into cylindrical lengths or sections which are dried and then impregnated with the water gas tar pitch, or the like, at a temperature above the melting point of the pitch but below the charring temperature of the pulp.

Our invention resides in an impregnating process in which an alternation of temperature or a plurality of temperature cycles are employed, which we find results in a marked increase in the waterproofing effect. To a certain extent there is also an increased absorption of the pitch, although this increase in pitch absorption is not in itself sufficient to account for the substantial increase in the waterproofing effect.

The alternation or cycle of temperature in the impregnating operation is preferably one in which initial and final temperatures are higher than one or more of the intermediate temperatures of treatment, but good results are not dependent on

this particular temperature relation, and the treatment may start or end with a lower temperature, or vice versa. The temperatures employed may range in the case of water gas tar pitch and newsprint pulp from about 300° F. to 450° F. and we find that three or four alternations of temperature over a period of as many hours are sufficient to give substantially the desired results, and that longer time or more alternations do not correspondingly improve the product. The temperature limits may obviously vary in accordance with the materials employed, for the reason that different fiber or pulp can withstand different temperatures without injury, and different impregnating substances will have different melting points and viscosities. Furthermore, many of the impregnating compounds or mixtures have volatile components, so that the upper temperature limit will depend somewhat upon the composition of the impregnating substance for this reason. The final temperature in the impregnating tanks is so chosen that proper drainage of the product will take place when the article is removed from the impregnating tank. This is of particular importance in the manufacture of fiber conduit and duct in order that the exterior surface will not retain an objectionable thickness of pitch over the pulp.

The following examples illustrate results obtained in treating newsprint pulp bodies with water gas tar pitch, in accordance with the invention and by the ordinary method.

|                                                | Percent saturation | Water absorption 120 hrs. 37° C. | 85 |
|------------------------------------------------|--------------------|----------------------------------|----|
| 5 changes—4½ hrs. 480-350° F. Not transferred. | 80%                | 2%                               |    |
| 4 changes—4 hrs. 450-300° F. Not transferred.  | 80-82%             | 3-6%                             |    |
| Uniform temperature—4 hrs.—350° F. -----       | 75-79%             | 9-14%                            | 90 |

The above figures show plainly the greater absorption of the pitch and the greatly improved waterproofing obtained by the alternation of temperature as compared with treatment at a uniform temperature for approximately the same time. The articles treated in these examples were left in the tank while the temperature changes were being effected.

The following figures were obtained under somewhat different conditions of temperature and time, as indicated in the table, the articles being transferred from one tank to the other in 5 the treatment at alternating temperatures.

|                                                            | Percent saturation | Water absorption 120 hrs.—37° C. |
|------------------------------------------------------------|--------------------|----------------------------------|
| 10                                                         |                    |                                  |
| Uniform at 300° F.                                         | 78.6%              | 13.3%                            |
| Uniform at 350° F.                                         | 75.1%              | 16.0%                            |
| Uniform at 400° F.                                         | 74.1%              | 14.8%                            |
| Uniform at 450° F.                                         | 74.4%              | 12.4%                            |
| 15 Alternating 300-450 (transferring) 4 hrs.—eight changes | 77.6%              | 6.4%                             |

It might ordinarily be supposed that increasing temperature would represent a decreased weight percentage of pitch saturation, due to the lower density of the pitch at the elevated temperature, and that the lower temperature alone would therefore represent the greatest weight percentage of pitch absorbed. The above figures, however, show that the relation is complex in 20 that the percentage of pitch saturation decreases steadily with increases in temperature under the uniform temperature treatment, whereas the alternating temperature treatment gives a percentage of saturation almost equivalent to the saturation obtained at the lowest uniform temperature treatment. The waterproofing quality is shown to be much greater in 25 the alternating temperature treatment than that obtained at the lowest uniform temperature treatment, although the latter represented a greater percentage of absorption of the pitch. The results indicate that increasing temperature alone in the uniform temperature treatment tends to decrease the amount of pitch absorption, although it may improve the waterproofing quality. The alternating treatment does not 30 substantially reduce the weight percentage of pitch absorption, but very greatly improves the waterproofing quality.

35 40 45 The following table represents results obtained on impregnating newsprint pulp duct with various substances under specified conditions, the product being removed from the final treatment at 350° F., in each test.

| 50 | Saturation                                                  | Water absorption |                          |                 | 125    |     |
|----|-------------------------------------------------------------|------------------|--------------------------|-----------------|--------|-----|
|    |                                                             | 37° C. 120 hrs.  | 37° C. 1 month immersion | 37° C. 6 months |        |     |
| 55 |                                                             |                  |                          |                 | 130    |     |
|    | <i>Pitch</i>                                                |                  |                          |                 |        |     |
| 60 | Maintained uniformly at 350° F. 4 hours                     | 66-68%           | 13.0%                    | 20.0%           | 135    |     |
| 60 | Alternating 300-450° F. 4 changes 4 hours (not transferred) | 70-73%           | 1.5%                     | 3.5%            | 7.3%   | 135 |
| 65 | <i>Stanolite (an asphaltic material)</i>                    |                  |                          |                 |        |     |
| 65 | Maintained uniformly at 350° F. 4 hours                     | 66-70%           | 10.0%                    | 17.7%           | 26.6%  | 140 |
| 65 | Alternating 300-450° F. 4 changes 4 hours (not transferred) | *68.5%           | 4.1%                     | 6.2%            | 12.1%  | 140 |
| 70 | <i>Stanolite+varying amounts of wax tallings up to 5%</i>   |                  |                          |                 |        |     |
| 70 | Maintained uniformly at 350° F. 4 hours                     | 65-68%           | 7-11%                    | 12-19%          | 20-34% | 145 |
| 70 | Alternating 300-450° F. 4 changes 4 hours (not transferred) | 67-70%           | 2-5%                     | 4-6%            | 9-10%  | 145 |

75 \*In this case no greater saturation obtained.

The above series of results are particularly interesting in that they show much more pronounced effects after long time immersion up to six months than is evident in the short period immersion test (120 hours), favorable as the latter are. These results show, also, the fact that the increase in water resistance is out of all proportion to slight increases in the saturation.

The fact that the principal gain, as compared with the ordinary method of impregnation, is obtained in a relatively few cycles of temperature changes, after which the slight additional gain may not be commercially economical, is shown by tests in which samples were treated for 4 hours total time between temperatures of 300° F. and 400° F., with a like period of time at each of the temperatures stated, namely, 300° F. then 400° F., showing in the treated sample a water absorption of 13.5%, 400° F. then 300° F. then 400° F., showing in the sample treated a water absorption of 6.1%, and treatment at 400° F. then 300° F. then 400° F. then 300° F. and finally 400° F., showing in the treated sample a water absorption of 5%.

We claim:—

1. The method of impregnating a porous body which comprises the immersion treatment of the body with an impregnating material for substantial time periods first at one temperature, then at another temperature, and again at the first temperature, each of said temperatures being above the melting point of the impregnating material.

2. The method of impregnating a porous body which comprises the immersion treatment of the body with an impregnating material at one temperature, continuing the treatment at a lower temperature, and repeating the treatment at a higher temperature, each of said treatments being for a substantial time period and at a temperature above the melting point of the impregnating material.

PHILIP P. GRAY.  
ERNEST E. WERLE.

120

125

130

135

140

145

150